

United States Patent [19]  
Watanabe et al.

[11] 3,895,974  
[45] July 22, 1975

- [54] **PROCESS FOR PRODUCING A GRAIN-ORIENTED ELECTRICAL STEEL SHEET HAVING EXCELLENT MAGNETIC CHARACTERISTIC**
- [75] Inventors: **Shozo Watanabe, Tokyo; Kiyoshi Tanaka; Yozo Suga**, both of Himeji, all of Japan
- [73] Assignee: **Nippon Steel Corporation**, Japan
- [22] Filed: Oct. 3, 1973
- [21] Appl. No.: 402,908
- [30] **Foreign Application Priority Data**  
Oct. 11, 1972 Japan ..... 47101795
- [52] U.S. Cl. ..... 148/111; 148/31.55; 148/112; 148/120; 148/121
- [51] Int. Cl. ..... H01f 1/04
- [58] **Field of Search** ..... 148/111, 112, 110, 120, 148/121, 122, 31.55

| References Cited      |         |                    |         |
|-----------------------|---------|--------------------|---------|
| UNITED STATES PATENTS |         |                    |         |
| 2,084,337             | 6/1937  | Goss .....         | 148/111 |
| 3,144,363             | 8/1964  | Aspden et al. .... | 148/111 |
| 3,671,337             | 6/1972  | Kumai et al. ....  | 148/111 |
| 3,764,406             | 10/1973 | Littmann .....     | 148/111 |

*Primary Examiner*—Walter R. Satterfield  
*Attorney, Agent, or Firm*—Toren, McGeady and Stanger

[57] **ABSTRACT**

A process for producing a high magnetic flux density grain-oriented electrical steel sheet having at least more than 1.85 Wb/m<sup>2</sup> by subjecting a silicon steel containing not less than 2% Si, 0.010 to 0.045% so-1.Al, 0.0030 to 0.0080% total N, and unavoidable impurities to a light hot working immediately after the hot rolling or prior to the cold rolling to precipitate AlN.

2 Claims, 6 Drawing Figures

FIG. 1



FIG. 2



FIG. 3



PATENTED JUL 22 1975

3,895,974

SHEET

3

Fig. 6



Fig. 5



Fig. 4



# PROCESS FOR PRODUCING A GRAIN-ORIENTED ELECTRICAL STEEL SHEET HAVING EXCELLENT MAGNETIC CHARACTERISTIC

The present invention relates to a process for producing so-called grain-oriented electrical steel sheets having a magnetizable axis <100> in the rolling direction.

Silicon steels widely used presently as materials for the grain-oriented electrical steel sheets are composed of grains having a body-centred cubic lattice, and it is well known that the direction <100> along the three tetragonal axis is most easily magnetized. The grain-oriented electrical steel sheet is a steel sheet in which this magnetizable axis <100> is arranged in the rolling direction and the plane {110} is arranged in parallel to the rolling plane, and crystallographically it is referred to as (110)[001] orientation by the Miller indices.

As above explained, the grain-oriented electrical steel sheet is composed of the grains having the specific selective orientation, and such grain orientation is attained by the secondary recrystallization phenomenon during the final annealing of the cold rolled steel sheet of final thickness.

The grain-oriented electrical steel sheets are used mainly as iron cores for transformers and other electrical appliances, and they must have good exitation and low watt loss characteristics as magnetic properties.

In the present invention, as the value representing the exitation characteristics, the magnetic flux density  $B_s$  ( $\text{Wb}/\text{m}^2$ ) produced in the iron core at an intensity of the magnetic field  $H = 800\text{A}\cdot\text{T}/\text{m}$  (ampere per meter) is used, and the value for representing the energy loss caused when predetermined A.C magnetic flux density is given to the iron core, namely the watt loss, the watt loss at A.C magnetic flux density of  $1.7\text{ Wb}/\text{m}^2$  and 50 Hz frequency is used.

In recent years, tendencies have been toward enlarged sizes of the electrical appliances and trials have been made for increasing the magnetic flux density value and for decreasing the weight of the iron core in view of the restrictions in transportation and others. For this purpose, an electrical steel sheet showing excellent magnetic characteristics in a high magnetic flux density zone has been demanded.

Therefore one of the objects of the present invention is to provide a process for producing an electrical steel sheet which satisfies the above requirements.

According to the present invention, it is possible to produce a high magnetic flux density grain-oriented electrical steel sheet which shows a magnetic flux density  $B_s$  in the rolling direction of at least more than  $1.85\text{ Wb}/\text{m}^2$ .

More particularly, the present invention is to provide a process for producing grain-oriented electrical steel sheet having excellent magnetic characteristics by hot rolling a silicon steel material comprising not less than 2% preferably 2.0 to 4.5% silicon, 0.010 to 0.045% preferably 0.027 to 0.045% acid soluble aluminium (sol.Al), 0.0030 to 0.0095% preferably 0.0065 to 0.0095% nitrogen, with the balance being iron and unavoidable impurities, cold rolling the hot rolled material to the final sheet thickness and subjecting the cold rolled sheet to a high temperature annealing, which is characterized in that the hot rolled material is subjected to light hot working of 3 to 20% preferably 10 to 16% at a temperature between  $700^\circ$  and  $900^\circ\text{C}$  preferably  $720^\circ$  and  $830^\circ\text{C}$  and held in the temperature

range not shorter than 2 seconds prior to the cold rolling.

The silicon steel as the starting material of the present invention contains not less than 2% silicon 0.010 to 0.045% acid soluble aluminium and 0.0030 to 0.0095% total nitrogen and impurities usually contained in steels.

The chemical composition of the starting material of the present invention including the impurities is shown in Table 1, but the amounts of the impurities other than silicon, acid soluble aluminium and the total nitrogen should not be limited to the ranges shown in the table.

Table 1

| Elements | Contents         |
|----------|------------------|
| C        | 0.025 – 0.060%   |
| Si       | more than 2%     |
| Mn       | less than 0.15%  |
| P        | less than 0.025% |
| S        | less than 0.030% |
| Sol.Al   | 0.010 – 0.045%   |
| T.N      | 0.0030 – 0.0080% |

As the present invention is directed to obtain a high grade electrical steel sheet having excellent magnetic properties at a high magnetic field, the silicon content is defined as not less than 2%.

As the dispersed precipitates utilized to obtain grain-oriented electrical sheets through the secondary recrystallization in the present invention, AlN is mainly utilized, and thus the amounts of acid soluble aluminium and total nitrogen which form AlN are particularly defined.

Regarding the content of acid soluble aluminium, with less than 0.010% acid soluble aluminium, the amount of AlN is not enough to be utilized as the dispersed precipitates. On the other hand, if the content of acid soluble aluminium is beyond 0.045%, uniformity in the refinement of the dispersed precipitates of AlN is damaged. Therefore the content of acid soluble aluminium is limited to 0.010 to 0.045%.

As for the content of the total nitrogen, if the total nitrogen is less than 0.0030%, the amount of AlN is not enough as in the case of the acid soluble aluminium and if the total nitrogen is over 0.0095%, there will be caused in the final product surface defects such as commonly called blisters. Therefore, the total nitrogen content is limited to 0.0030 to 0.0095%.

According to the present invention, the silicon steel as shown in Table 1 is used as starting material, and is subjected to a light hot working immediately after the hot rolling or prior to the cold rolling to obtain appropriate precipitation of AlN, thereby a high magnetic flux density grain-oriented electrical steel sheet having at least more than  $1.85\text{ Wb}/\text{m}^2$  of flux density  $B_s$  can be produced.

It is disclosed in a Japanese Pat. No. Sho 40-15644 to utilize AlN as the dispersed precipitate for the secondary recrystallization and to adjust the precipitation of AlN prior to the cold rolling for the production of a high magnetic flux density grain-oriented electrical steel sheet.

However, the precipitation treatment of AlN in the above prior art is conducted by a high temperature heat treatment between  $900^\circ$  and  $1,200^\circ\text{C}$  for 30 seconds to 30 minutes. This is completely different from the pres-

ent invention in which the precipitation of AlN is made uniform by the light hot working.

According to the present invention, the light hot working is conducted in a temperature range in which the precipitation of AlN takes place suddenly to disperse the precipitation sites thereby finely and uniformly dispersed precipitates of AlN most suitable to the secondary recrystallization is rapidly obtained. Thus the present invention is based on technical thought completely different from the precipitation treatment of AlN conducted after the light cold working, or the simple precipitation treatment of AlN without a light working.

Further, in order to conduct the precipitation treatment of AlN according to the prior art Japanese Pat. No. Sho 40-15644, a heat treatment equipment capable to conduct the high temperature heat treatment is required, whereas in the present invention, the AlN precipitation conditions can be obtained immediately after the continuous hot rolling only by adding special conditions in the ordinary continuous hot rolling mill. Thus the present invention is advantageous in economical aspects, too.

The present invention will be described in detail by referring to the attached drawings.

FIG. 1 is a graph showing the relation among the light hot rolling temperature the rolling reduction rate and the  $B_{\text{H}}$  value.

FIG. 2 is a graph showing the relation among the bending ratio, the bending temperature and the  $B_{\text{H}}$  value.

FIG. 3 is a graph showing the relation between the holding time after the light hot working and the  $B_{\text{H}}$  value.

FIG. 4 to FIG. 6 are electron microscopic photographs showing the precipitation of AlN.

FIG. 1 shows the magnetic flux density of a specimen which was prepared by heating rapidly hot rolled steel plate of 2.3mm thickness containing 2.95% Si, 0.025% sol.Al, 0.0058% total N to a temperature between 700° and 1,100°C, giving the plate a light rolling of 0 to about 26%, holding the plate for 4 seconds, quenching the plate in a salt water, cold rolling the plate to 0.30mm thickness, decarburizing the sheet in a wet hydrogen atmosphere, and subjecting the sheet to a high temperature annealing for the secondary recrystallization.

As clear from FIG. 1, a grain-oriented electrical steel sheet having high magnetic flux density can be obtained by conducting the light hot working at a temperature between 700° and 1,100°C with a reduction rate between 3 and 20%, and the light hot working conditions of the present invention have been defined on the basis of the above experiments.

The results shown in FIG. 1 were obtained by adopting the hot rolling as the light hot working, but the light hot working can be conducted by any of other equipments which can give the specified reduction rate such as roller levellers, stretcher levellers and so on.

For example, FIG. 2 shows the magnetic flux density of a specimen prepared by rapidly heating the hot rolled steel sheet as used in FIG. 1 to a temperature between 500° and 1,000°C, bending the sheet with bending radius of 25mm and 50mm, holding the sheet for 4 seconds, quenching the sheet in a salt water and then treating the sheet in a similar way as in FIG. 1.

The maximum working ratios corresponding to the bending ratios of 25mm and 50mm are 4.4% and 2.3% respectively, and it is understood that the desired results of the present invention can be obtained if the temperature and the working ratio for the light hot working are satisfied irrespective to the kind of the light hot working.

The other feature of the present invention is to obtain an appropriate precipitation of AlN by the light hot working, and for this purpose a certain holding time is required for changing the AlN precipitation.

FIG. 3 shows magnetic flux densities of five specimens prepared by rapidly heating to 800°C five hot rolled steel sheets of 2.3mm thickness containing 2.5 to 3.2% Si, 0.015 to 0.025% sol.Al, and 0.0050 to 0.0070% total N, subjecting the sheets to light hot rolling of 9.5 to 10.5%, holding the sheets at various times after the light hot rolling to the quenching in a salt water (the temperature of the sheets after the light hot rolling was about 750°C), quenching the sheets in a salt water, cold rolling the sheets to 0.30mm thickness and subjecting the sheets to decarburization annealing and high temperature annealing. The results show that the object of the present invention is attained by the holding times not shorter than 2 seconds.

Further, according to the present invention, AlN is utilized as the dispersed precipitates for the secondary recrystallization and the light hot working is utilized for rendering the AlN precipitates into an appropriate form. The present inventors have conducted studies on effects of the light hot working on the form of AlN precipitates.

Samples were taken from the specimens used in FIG. 1 at each of the steps and subjected to chemical analysis and electron microscope observation.

Table 2

| Sampl-<br>es | Hot Rolled<br>Steel<br>Plate | Changes of AlN |     |       |     |       |     |
|--------------|------------------------------|----------------|-----|-------|-----|-------|-----|
|              |                              | 700°C          |     | 800°C |     | 900°C |     |
|              |                              | 0%             | 11% | 0%    | 11% | 0%    | 10% |
| N as<br>AlN  | 28                           | 47             | 52  | 48    | 51  | 49    | 52  |

Figures in Table 2 show N as AlN (amount of N precipitated as AlN). Unit:  $\times 10^{-4}\%$ .

As shown in Table 2, the amount of AlN in the hot rolled steel sheets remarkably increases when the sheets were heated to respective temperatures irrespective to the light hot working. (In actual, the amount is slightly larger when the light hot rolling is done.)

However, according to the observation by the electron microscope, clear differences are observed in the AlN precipitates between the sheet subjected to the light hot working and the one subjected to no such working.

Namely, FIG. 4 shows the distribution of AlN in the hot rolled sheet, FIG. 5 shows the sheet which was heated rapidly to 800°C and cooled without the light hot rolling, and FIG. 6 shows AlN in the sheet which was heated rapidly to 800°C and subjected to light hot rolling of 11%.

As is understood from the comparison of FIG. 4 to FIG. 6, AlN precipitates finely and uniformly when the light hot rolling is conducted. On the other hand, when the light hot rolling is not conducted, the AlN precipi-

tates are in flocks, resulting in irregular distribution of AlN.

Therefore, it is assumed a grain-oriented electrical steel sheet having a high magnetic density flux can be obtained by the light hot working in the present invention due to the fact that the finely and uniformly precipitated AlN formed by the light hot working has remarkable effects on the cold rolling or on the primary recrystallization structure or on the secondary recrystallization phenomenon.

The present invention will be more clear from the following examples.

#### EXAMPLE 1

Twelve silicon steel slabs (180mm thick) containing 3.05% Si, 0.023% sol. Al, 0.0063% total N and unavoidable impurities were hot rolled to 2.25mm thickness by a continuous hot rolling mill and comparison tests were conducted under the following conditions shown in Table 3.

Table 3

| Conditions            | Conditions of hot rolling and cooling |                                                                              |                                                                              |
|-----------------------|---------------------------------------|------------------------------------------------------------------------------|------------------------------------------------------------------------------|
|                       | Methods                               | Conventional                                                                 | Inventive                                                                    |
| Final Stand           | Reduction Rate<br>Speed               | 10%<br>550 mpm                                                               | 10%<br>550 mpm                                                               |
| Finishing Temperature |                                       | 830 – 850°C                                                                  | 830 – 850°C                                                                  |
| Cooling Conditions    |                                       | Water cooling started 10m after the outlet of the final stand (about 1 sec.) | Water cooling started 40m after the outlet of the final stand (about 4 sec.) |
| Cooling Temperature   |                                       | Not higher than 500°C                                                        | Not higher than 500°C                                                        |

Then the hot rolled steel strips were cold rolled to 0.30mm thickness, subjected to decarburizing annealing in wet hydrogen at 830°C for 3 minutes and a high temperature annealing at 1,200°C for 20 hours to obtain grain-oriented electrical steel sheets.

The magnetic characteristics of the electrical steel sheets thus obtained are shown in Table 4.

Table 4

| Magnetic Characteristics                         | Magnetic Characteristics                  |                                                 |           |
|--------------------------------------------------|-------------------------------------------|-------------------------------------------------|-----------|
|                                                  | Cooling Conditions of Hot Rolled Strips   | Conventional                                    | Inventive |
| Magnetic Characteristics                         | Cooling started 10m after the final stand | Cooling started after 40m after the final stand |           |
| Watt Loss W 17/50 (W/Kg)                         | 1.423 (1.34 – 1.52)                       | 1.198 (1.12 – 1.25)                             |           |
| Flux Density B <sub>s</sub> (Wb/m <sup>2</sup> ) | 1.764 (1.73 – 1.82)                       | 1.893 (1.86 – 1.93)                             |           |

Measurement was done at 12 points (25cm Epstein samples)

As seen from the results shown in Table 4, the magnetic characteristics are remarkably improved by application of the present invention to the conventional continuous rolling hot rolling mill.

#### EXAMPLE 2

The hot rolled steel strips obtained by the conventional method and used in Example 1 were subjected to a light hot rolling as shown in Table 5, cold rolled and subjected to decarburizing annealing and a high temperature annealing to obtain electrical steel sheets of 0.30mm thickness.

Table 5

| Temperature | Reduction Rate | Holding Time | Light Hot Rolling Conditions and Magnetic Characteristics |                                      |
|-------------|----------------|--------------|-----------------------------------------------------------|--------------------------------------|
|             |                |              | Watt Loss W 17/50                                         | Magnetic Flux Density B <sub>s</sub> |
| 600°C       | 0              | 3 sec.       | 1.48                                                      | 1.74                                 |
|             | 10.5           | 3            | 1.40                                                      | 1.77                                 |
|             | 11.0           | 1            | 1.43                                                      | 1.76                                 |
|             | 0              | 3            | 1.41                                                      | 1.76                                 |
| 850°C       | 5.5            | 3            | 1.21                                                      | 1.89                                 |
|             | 10.0           | 3            | 1.12                                                      | 1.92                                 |

|               |     |      |      |
|---------------|-----|------|------|
| 10.5          | 0.5 | 1.33 | 1.83 |
| 0             | 3   | 1.54 | 1.73 |
| 9.5           | 3   | 1.34 | 1.83 |
| 10.0          | 1.5 | 1.37 | 1.79 |
| As hot rolled |     | 1.43 | 1.75 |

Units: Watt Loss – W/Kg, Magnetic Flux Density – Wb/m<sup>2</sup>.

From the relation between the light hot rolling conditions and the magnetic characteristics shown in Table 5, it is clear that remarkable improvement of the magnetic characteristics can be obtained by application of the present invention to the hot rolled steel strips.

What is claimed is:

1. A process for producing a goss texture, grain-oriented electrical steel sheet having excellent magnetic characteristics greater than 1.85 Wb/m<sup>2</sup> comprising hot rolling a silicon sheet material consisting essentially of not less than 2% silicon, 0.01 to 0.45% acid soluble aluminium, 0.003 to 0.0095% nitrogen with the balance being iron and unavoidable impurities, cold rolling the hot rolled material to a final sheet thickness, subjecting the cold rolled sheet to decarburization annealing and further subjecting the sheet to a final annealing in a temperature range where the secondary recrystallisation proceeds in the presence of aluminium nitride as it exists in the steel sheet thus produced, wherein the hot rolled sheet is subjected to a light hot working of 3 to 20% in a temperature range between

700° to 900°C and is held in this temperature range for not less than 2 seconds prior to the cold rolling to precipitate aluminium nitride which is effective for the secondary recrystallisation at the stage of final annealing.

2. A process according to claim 1, wherein the silicon

steel material consists essentially of 2.0 to 4.5% silicon, 0.027 to 0.045% acid soluble aluminium, 0.0065 to 0.0095% nitrogen, and the light hot working is performed with a reduction rate between 10 and 16% at 5 a temperature between 720° and 830°C.

\* \* \* \* \*

10

15

20

25

30

35

40

45

50

55

60

65